# EUROPEAN PATENT SPECIFICATION

(11) **EP 0 518 905 B1**
(45) Date of publication and mention of the grant of the patent: **29.06.1994**
(21) Application number: 91904935.3
(22) Date of filing: 05.03.1991
(51) Int. Cl.: G03C 7/42, G03C 7/44, G03C 5/395

(54) **SILVER REMOVAL FROM PHOTOGRAPHIC PRODUCTS**
SILBERENTFERNUNG AUS PHOTOGRAPHISCHEN PRODUKTEN
RECUPERATION DE L'ARGENT DES PRODUITS PHOTOGRAPHIQUES

(30) Priority: 07.03.1990 GB 9005130
(43) Date of publication of application: 23.12.1992
(73) Proprietor: KODAK LIMITED, Hemel Hempstead Hertfordshire HP1 1JY (GB); EASTMAN KODAK COMPANY, Rochester, New York 14650-2201 (US)
(72) Inventor: FYSON, John, Richard, Kodak Ltd., Kodak House, Herts HP1 1JY (GB)
(74) Representative: Stebbing, Peter John Hunter
(86) International application number: EP9100406
(87) International publication number: WO9114205

(56) References cited:
- EP-A- 0 173 540
- EP-A- 0 213 710
- GB-A- 1 138 842
- GB-A- 1 150 466
- GB-A- 1 411 985
- US-A- 4 293 639
- PATENT ABSTRACTS OF JAPAN vol.001,no.136(E-062) 10 November 1977,& JP-A-52 073033
- PATENT ABSTRACTS OF JAPAN vol.11,no.276(P-613)(2723)08 September 1987,&JP-A-62 075525

## Description

The present invention relates to improvements in silver removal from photographic products, and particularly from developed photographic materials to enable successful silver removal during a bleach-fix step.

It is common to use a bleach step followed by a fix step, optionally with a washing step between to remove silver from images in negative photographic products. With print materials such as colour photographic paper the bleach can be combined with the fix to give a bleach-fix composition. However the silver removing power of this bleach-fix composition is insufficient to remove all silver from camera speed materials. This is believed to be caused by inhibiting materials absorbed onto the developed silver surface.

Thus one problem in the art is to remove the inhibiting absorbed materials from the developed silver surface, of the photographic product whether positive or negative.

Another problem lies with silver recovery. It is common to remove silver from used photographic reagents. This is usually effected as a separate step either chemically or electrolytically. This recovery progress is more easily effected from the fix step rather than the bleach-fix step, and further it would be most desirable if silver recovery could be effected, in a large part at least, as a function of the silver removal process from the photographic material rather than as a separate removal process.

These problems have in part been addressed in US-A-3,893,858. In this disclosure an accelerator selected from certain aliphatic thiols is used to assist silver removal. These thiols may be selected from compounds containing a thio-group in combination with one or more solubilizing groups.

Further EP-A-0,173,540 reveals dimethyl and diethyl aminoalkylenethiols but not the compounds as defined.

We have now found however that where the accelerators are used per se as a prebath prior to the bleach-fix step, their useful life is not long enough to be commercially worthwhile, whereas if the accelerator is added to the bleach-fix there is a tendancy for the accelerator to cause staining as a result of the accelerator reacting with itself in the bleach-fix on standing. For these reasons the use of accelerators has not been common in the art over the last few years.

We have now found that these stability problems may be addressed by adding the accelerator to the fixer which produces the bleach-fix. This has two effects; first it stabilizes the accelerator thereby to increase its active life, and second the stabilizing effect alleviates any subsequent staining problems. More importantly however silver removal may be effected at the fixer stage.

Accordingly the inclusion of the accelerator in the fixer has the effect of promoting product quality while allowing effective silver removal from the fixer stage thereby, with care, allowing the silver recovery without the previously required separate silver recovery step.

In a preferred embodiment in accordance with the invention the silver recovery is effected by precipitation of a silver product as a result of an intereaction of the accelerator with a silver complexed species which can be readily recovered, by usual methods of solid/liquid separation such as filtration.

According therefore to a first aspect of the present invention there is provided a method for photographic processing in which an image-wise exposed and colour developed photographic element is contacted with a fixing agent, wherein said element is also contacted with an accelerator selected from a bleach accelerating amount of a thiol or a photographically effective salt thereof, said thiol being selected from monothioglycerol, cystine, cystamine, cysteine, and aminoalkylenethiols of the formula:
wherein each of R¹ and R² is individually H, CH₃ or C₂H₅ with the proviso that at least one of R¹ or R² is H, and n is an integer having a value of 1 to 3; prior to contact with a bleach-fix agent to oxidize metallic silver and remove the same from the element;
characterised in that the accelerator is present as part of the fixing agent composition.

In a preferred form of the invention the fixing agent comprises a thiosulphate or chemically analogous compound and the bleach-fix bath contains a ferric amino polycarboxylic acid.

In a further aspect of the present invention there is provided a method for the recovery of silver from a photographic process in which an image-wise exposed and colour developed silver containing photographic element is contacted with a fixing agent before contact with a bleach-fixing solution;
which recovery method comprises adding to the fixing agent an accelerator selected from monothioglycerol, cystine, cystamine, cysteine, and aminoalkylenethiols of the formula
in which R¹ and R² is each H, CH₃ or C₂H₅, with the proviso that at least one of R¹ or R² is H, and n is an integer having a value of 1 to 3;
thereby to cause the silver to precipitate as a silver salt and recovering said silver salt for reprocessing.

Preferably the bleach-fixing agent is a thiosulphate and the silver is removed as a precipitate of silver sulphide or silver thiol. Preferred accelerating agents in accordance with the present invention are monothioglycerol, cysteine and cystine.

The invention will now be described, by way of illustration only, with reference to the following Example, and with reference to the accompanying drawings wherein:

Figure 1 shows a graph of the sensitometry of kodacolor VR100 film processed through a standard C-41 process. This is compared to the same film processed through the example process.

Figure 2 shows a graph of the sensitometry of Kodacolor VR200 film processed through a standard C-41 process. This is compared to the same film processed through the example process.

Figure 3 shows a graph of the sensitometry of Kodacolor VR400 film processed through a standard C-41 process. This is compared to the same film processed through the example process.

Figure 4 shows a graph of the sensitometry of Kodacolor VR1000 film processed through a standard C-41 process. This is compared to the same film process through the example process.

These figures demonstrate that the process has little or no effect on the final sensitometry i.e. a film processed through the control process would be undistinguishable from an image point of view from one processed in a standard C-41 process.

### EXAMPLE

A fix was prepared according to the following formula using commercially available materials:

### Experimental Accelerating Fix.

The pH of this solution was adjusted to 6.5 by the addition of acetic acid.

A bleach-fix was prepared according to the following formula using commercially available materials:-

### Experimental Bleach-fix.

The pH of this solution was adjusted to 6.0 by the addition of acetic acid.

A developer, bleach and fix were made up using Kodak C-41 20 litre kits according to the instructions enclosed in the kit boxes.

Strips of four Kodak colour negative films, VR100, VR200, VR400, VR1000 were exposed to simulated daylight through a 0.2 log exposure sensitometric wedge for 0.01 seconds. These strips were kept for 24 hours then processed through the following process:

Similar strips of exposed and aged film were processed in a standard C-41 process as described in the C-41 manual. The processed strips were measured using a Macbeth densitometer and compared. Figures 1-4 show the results for the four different films. The levels of residual silver in all strips Dmaxs were all less than could be detected with any confidence by X-ray Fluorescence Spectroscopy i.e. 25mg/sq.m.

The experiment was repeated with a number of other compounds in place of the DMAET in the experimental fix, all used at a concentration of 5g/l. Table 1 below shows the red, green and blue Dmax densities of the four films processed in the experimental process with the different experimental fixes, using the experimental fixes, using the experimental bleach-fix for 2′00˝ in all cases.

In those films thet had been processed with an additive present in the fix, no silver could be detected by infra-red density measurements.

## Claims

1. A method for photographic processing in which an image-wise exposed and colour developed photographic element is contacted with a fixing agent, wherein said element is also contacted with an accelerator selected from a bleach accelerating amount of a thiol or a photographically effective salt thereof, said thiol being selected from monothioglycerol, cystine, cystamine, cysteine, and an aminoalkylenethiol of the formula wherein each of R¹ and R² is individually H, CH₃ or C₂H₅, with the proviso that at least one of R¹ and R² is H, and n is an integer having a value of 1 to 3; prior to contact with a bleach-fix agent to oxidize metallic silver and remove the same from the element;
characterised in that the accelerator is present as part of the fixing agent composition.

2. A method according to claim 1 characterised in that the fixing agent contains a thiolsulphate and the bleach-fix agent contains a ferric amino polycarboxylic acid.

3. A method according to either of claims 1 or 2 characterised in that the accelerator is selected from thioglycerol cysteine and cystine.

4. A method according to either of claims 2 or 3 characterised in that the ratio by weight of accelerator to the thiosulphate in the fixer bath is 1 to 2:100.

5. A method for the recovery of silver from a photographic process in which an image-wise exposed and colour developed silver containing element is contacted with a fixing agent before contact with a bleach-fixing solution; which recovery method comprises adding to the fixing agent an accelerator selected from monothioglycerol, cystine, cystamine, cysteine, and an aminoalkylenethiols of the formula: wherein each of R¹ and R² is individually H, CH₃ or C₂H₅ with the proviso that at least one of R¹ and R² is H, and n is an integer having a value of 1 to 3;
thereby to cause the silver to precipitate as a silver salt and recovering said silver salt for reprocessing.

6. A method according to claim 5 characterised in that the fixing agent contains a thiosulphate and the bleach-fix stage contains a ferric amino carboxylic acid.

7. A method according to either of claims 5 or 6 characterised in that the accelerator is selected from monothioglycerol, cysteine and cystine.

8. A method according to either of claims 6 or 7, characterised in that the weight ratio of accelerator to the thiosulphate in the fixer bath is 1 to 2:100.

## Patentansprüche

1. Verfahren zur photographischen Verarbeitung, bei dem ein bildweise belichtetes und farbentwickeltes photographisches Element mit einem Fixiermittel in Kontakt gebracht wird, wobei das Element auch mit einem Beschleuniger in Kontakt gebracht wird, der aus einer das Bleichen beschleunigenden Menge eines Thiols oder eines photographisch wirksamen Salzes hiervon gewählt wird, wobei das Thiol unter Monothioglycerin, Cystin, Cystamin, Cystein und Aminoalkylenthiolen der Formel ausgewählt wird,
worin R¹ und R² jeweils unabhängig H, CH₃ oder C₂H₅ bedeuten, mit der Maßgabe, daß wenigstens einer der Substituenten R¹ und R² H ist, und n eine ganze Zahl von 1 bis 3 ist,
und zwar vor dem Kontakt mit einem Bleichfixiermittel zum Oxidieren von metallischem Silber und Entfernen des Silbers aus dem Element,
dadurch **gekennzeichnet**,
daß der Beschleuniger als Teil der Fixiermittelzusammensetzung vorliegt.

2. Verfahren nach Anspruch 1, dadurch gekennzeichnet, daß das Fixiermittel ein Thiosulfat und das Bleichfixierbad eine Eisen(III)-aminopolycarbonsäure enthalten.

3. Verfahren nach Anspruch 1 oder 2, dadurch gekennzeichnet, daß der Beschleuniger unter Thioglycerin, Cystein und Cystin ausgewählt wird.

4. Verfahren nach Anspruch 2 oder 3, dadurch gekennzeichnet, daß das Gewichtsverhältnis von Beschleuniger zu Thiosulfat im Fixierbad 1 bis 2:100 beträgt.

5. Verfahren zur Rückgewinnung von Silber aus einem photographischen Prozeß, bei dem ein bildweise belichtetes und farbentwickeltes silberhaltiges Element vor dem Kontakt mit einer Bleichfixierlösung mit einem Fixiermittel in Berührung gebracht wird, wobei dem Fixiermittel ein Beschleuniger zugesetzt wird, der unter Monothioglycerin, Cystin Cystamin, Cystein und Aminoalkylenthiolen der folgenden Formel ausgewählt wird: worin R¹ und R² jeweils unabhängig H, CH³ oder C₂H₅ bedeuten, mit der Maßgabe, daß wenigstens einer der Substituenten R¹ und R² H ist, und n eine ganze Zahl von 1 bis 3 ist,
wodurch das Silber als Silbersalz ausgefällt und das Silbersalz für die Wiederverarbeitung zurückgewonnen wird.

6. Verfahren nach Anspruch 5, dadurch gekennzeichnet, daß das Fixiermittel ein Thiosulfat und die Bleichfixierlösung eine Eisen(III)-aminocarbonsäure enthalten.

7. Verfahren nach Anspruch 5 oder 6, dadurch gekennzeichnet, daß der Beschleuniger unter Monothioglycerin, Cystein und Cystin ausgewählt wird.

8. Verfahren nach Anspruch 6 oder 7, dadurch gekennzeichnet, daß das Gewichtsverhältnis von Beschleuniger zu Thiosulfat im Fixierbad 1 bis 2:100 beträgt.

## Revendications

1. Procédé pour le traitement photographique dans lequel un élément photographique exposé sous forme d'image est développé en couleur et mis en contact avec un agent de fixage, procédé dans lequel cet élément est également mis en contact avec un accélérateur choisi parmi une quantité accélérant le blanchiment d'un thiol ou de son sel efficace photographiquement, ce thiol étant choisi parmi le monothioglycérol, la cystine, la cystamine, la cystéine, et un aminoalkylènethiol de la formule dans laquelle chacun de R¹ et R² est individuellement H, CH₃ ou C₂H₅ sous réserve qu'au moins l'un de R¹ et R² est H, et n est un nombre entier ayant une valeur de 1 à 3, avant de mettre en contact un agent de fixage-blanchiment pour oxyder l'agent métallique et enlever celui-ci de l'élément, caractérisé en ce que l'accélérateur est présent comme partie constituante de la composition de l'agent de fixage.

2. Procédé selon la revendication 1, caractérisé en ce que l'agent de fixage contient un thiosulfate et l'agent de fixage-blanchiment contient un acide amino polycarboxylique ferrique.

3. Procédé selon l'une quelconque des revendications 1 ou 2, caractérisé en ce que l'accélérateur est choisi parmi la thioglycérol cystéine et la cystine.

4. Procédé selon l'une quelconque des revendications 2 ou 3, caractérisé en ce que le rapport en poids de l'accélérateur et du thiosulfate dans le bain de fixateur est de 1 à 2:100.

5. Procédé pour la récupération d'argent à partir d'un procédé photographique dans lequel un élément exposé sous forme d'image et contenant de l'argent développé en couleur est mis en contact avec un agent de fixage avant le contact avec une solution de fixage-blanchiment ; procédé de récupération qui comprend l'addition d'un accélérateur à l'agent de fixage, accélérateur choisi parmi la monothioglycérol, la cystine, la cystamine, la cystéine, et un aminoalkylènethiol de la formule dans laquelle chacun de R¹ et R² est individuellement H, CH₃ ou C₂H₅ sous réserve qu'au moins l'un de R¹ et R² est H, et n est un nombre entier ayant une valeur de 1 à 3,
faisant ainsi précipiter l'argent sous forme de sel d'argent et récupérer le sel d'argent pour le recyclage.

6. Procédé selon la revendication 5, caractérisé en ce que l'agent de fixage contient un thiosulfate et l'étape de fixage-blanchiment contient un acide amino carboxylique ferrique.

7. Procédé selon l'une ou l'autre des revendications 5 ou 6, caractérisé en ce que l'accélérateur est choisi parmi le monothioglycérol, la cystéine et la cystine.

8. Procédé selon l'une ou l'autre des revendications 6 ou 7, caractérisé en ce que le rapport pondéral entre l'accélérateur et le thiosulfate dans le bain de fixateur est de 1 à 2:100.
